

1

2,781,261

## PROCESS FOR THE MANUFACTURE OF TITANIUM-ALUMINUM ALLOYS AND REGENERATION OF INTERMEDIATES

Jonas Kamlet, Easton, Conn., assignor to National Distillers Products Corporation, New York, N. Y., a corporation of Virginia

No Drawing. Application October 30, 1953,  
Serial No. 389,503

13 Claims. (Cl. 75—135)

This invention relates to a process for the manufacture of titanium-aluminum alloys and the regeneration of the intermediates of said process. More particularly, it relates to a process for the manufacture of titanium-aluminum alloys containing from 0.1% to 95% of titanium, and for the processing of the by-products of said process to regenerate the intermediate chemical compounds required for the manufacture of said alloys.

Manchot and Richter (Annalen 357, 140—144 (1907)) reacted potassium fluotitanate with metallic aluminum in quantity far in stoichiometric excess of that required by the equation:



at advanced temperatures, and obtained a titanium-aluminum alloy containing 9.4% of titanium. In my co-pending application Serial No. 382,206, I have shown that alloys containing from 53% to 95% of titanium (the remainder being aluminum) may be obtained by the reaction, at advanced temperatures, of alkali metal fluotitanates with aluminum in quantities within a closely specified range. I now find that alloys of titanium and aluminum containing from 0.1% to 95% of titanium can be obtained by the reaction, at advanced temperatures, of alkali metal fluotitanates with metallic aluminum, employing per gram-mole of alkali metal fluotitanate (i. e. per 207.9 grams of  $\text{Na}_2\text{TiF}_6$ , or per 175.8 grams of  $\text{Li}_2\text{TiF}_6$ , or per 240.1 grams of  $\text{K}_2\text{TiF}_6$ ), from 38.5 grams to 47.9 kilograms of metallic aluminum.

This very broad range of titanium contents in the alloys obtained requires somewhat different modes of operating, depending on the melting point of the alloy to be prepared. The following chart represents the approximate melting point of the series of alloys preparable by the process of this invention:

| Percent Ti:              | Approximate melting point, °C. |
|--------------------------|--------------------------------|
| 0.1 to 1                 | 660 to 700                     |
| 5                        | 860                            |
| 10                       | 1020                           |
| 20                       | 1150                           |
| 30                       | 1280                           |
| 37.3 ( $\text{TiAl}_3$ ) | 1350                           |
| 40                       | 1370                           |
| 50                       | 1425                           |
| 60                       | 1440                           |
| 70                       | 1510                           |
| 80                       | 1600                           |
| 90                       | 1725                           |
| 95                       | 1730                           |

Binary alloys containing up to 37.28% of titanium consist of crystals of titanium aluminide ( $\text{TiAl}_3$ ) dispersed in excess aluminum. The binary alloy containing 37.28% of titanium corresponds to  $\text{TiAl}_3$  in composition. Binary alloys containing 37.28% to 53% of titanium consist of crystals of titanium aluminide dispersed in excess titanium metal. Binary alloys containing from 53% to 95% of

2

titanium comprise simple solutions of the aluminum in the titanium and do not form intermetallic compounds.

Formation of alloys containing up to 75% of titanium proceeds at a rapid rate. As a rule, the more aluminum that is used (within the limits above described), the more rapid and complete is the reaction between the alkali metal fluotitanate and the aluminum, and the formation of the titanium-aluminum alloy. As the amount of aluminum is decreased, the reaction with the alkali metal fluotitanate becomes slower, and there is a greater tendency for incomplete reduction of the alkali metal fluotitanate with formation of divalent and trivalent titanium compounds. By prolonged heating, however, alloys containing up to 95% titanium may however be obtained by this method.

The temperatures at which this reaction may be effected may vary quite widely. It is desirable to have at least one of the reagents (i. e. the aluminum) in a molten state, and preferably both the aluminum and the alkali metal fluotitanates should be in a molten state. Thus, the lower limit of temperature for this reaction is set by the melting point of aluminum, i. e. 660° C. Both reagents are molten in the range of 900°—1100° C. The upper limit of temperature for this reaction is set by the boiling point of aluminum (1800° C.) and the melting point of the alloy being prepared. It is desirable, at the conclusion of the reaction, to be able to separate a molten regulus of titanium-aluminum alloy from the concomitant "slag" consisting of molten alkali metal aluminum fluoride and aluminum fluoride. Thus, the temperature range for this reaction may be given as 660° C. to 1800° C., with a preferred range between 1100° C. and 1750° C., depending on the composition of the alloy being prepared.

A preferred method for effecting this step of the invention is to mix the calculated quantity of molten aluminum and alkali metal fluotitanate in a refractory-lined crucible in an induction furnace, and then to heat the mixture with agitation, if necessary, until the reaction is complete and a final temperature between 1100° C. and 1750° C. is obtained at which both the binary alloy and the salt mixture (i. e. the "slag") are molten. These two molten layers are then separated by decantation, in the usual manner, and each is then allowed to cool slowly and solidify. Magnesia-lined crucibles are, as a rule, suitable for the effecting of the reaction of this invention since they are not excessively attacked at the indicated reaction temperatures.

Although some of the alkali metal fluotitanates are known to form crystalline hydrates at lower temperatures, they are, of course, employed as anhydrous salts at the temperature ranges involved in the process of this invention. Since the aluminum is always employed in the molten state, it need not be comminuted prior to addition to the reaction mixture, but may be added to the crucible as bar or pig aluminum or in the molten state.

The titanium-aluminum alloys thus prepared have a wide range of utility in industrial metallurgy. They are employed to refine grain structure, remove gas occlusions, increase tensile strengths, increase resistance to leaking of castings, improve mechanical properties, decrease the electrical conductivity, increase impact resistance, increase resistance to acids, saline and other aggressive solutions, increase corrosion resistance, improve castings and lower the casting temperatures of various metals and alloys (Journ. Inst. Metals 1930, 531; Chem. Zintr. 1937I, 2002; 1944I, 242; Allumino 16, 5 (1947); U. S. Patents 2,252,421 and 2,376,681; Metallurtschaft 21, 683 (1942); Chimie & Industrie 26, 338 (1932); Aluminium 17, 79 (1934); 19, 635 (1937); 20, 452 (1938); 26, 2 (1944);

British Patent 473,916; Zeit. Anorg. Chem. 150, 26 (1926); Comptes rendus 220, 690 (1945); Journ. Metals 3 Trans. 1143 (1951).

In my co-pending patent application Serial No. 382,206, I also describe the use of alloys of titanium and aluminum containing from 53% to 95% of aluminum as intermediates in a process for the manufacture of titanium metal.

The by-product mixture of molten salts obtained with these titanium-aluminum alloys consists of substantially equimolecular proportions of alkali metal fluoaluminate ( $M_3AlF_6$ ) and aluminum fluoride. Since the starting material—the alkali metal fluotitanate—is not a common article of commerce, it is a further purpose of this invention to provide a simple process for the conversion of this by-product mixture of  $M_3AlF_6$  and  $AlF_3$  to the original starting material, i. e. the alkali metal fluotitanate— $M_2TiF_6$ .

I have found that this regeneration of the alkali metal fluotitanates may be effected by the following sequence of steps:

#### STEP A

The molten slag, comprising a substantially equimolecular mixture of alkali metal fluoaluminate and aluminum fluoride, obtained as above described, is cooled, comminuted and added to an aqueous slurry of milk of lime. The lime is used in stoichiometric proportions according to the equation:



(where M is an equivalent of an alkali metal), the reaction mixture is heated for a short period (e. g. 30 to 60 minutes) until precipitation of calcium fluoride is complete, and the insoluble calcium fluoride is then filtered from the residual aqueous solution comprising a solution of alkali-metal aluminates e. g. ( $Na_3AlO_3$  and  $3NaAlO_2$ ) ( $Na_2O/Al_2O_3$  ratio—1.5).

#### STEP B

The solution of alkali metal aluminates is then treated with a carbon dioxide-containing gas, until precipitation of aluminum hydroxide is complete, according to the equations:



This carbonation may be effected at ordinary or advanced temperatures and at atmospheric or superatmospheric pressures, according to the well known procedures of the art. The precipitate of aluminum hydroxide is then filtered or centrifuged from the aqueous solution of alkali metal carbonate (which may contain some bicarbonate when overcarbonated). The aluminum hydroxide may then be calcined (e. g. at 1000° C.) and converted to alpha-alumina for use in the electrolytic aluminum process. Alternatively, it may be used in the manufacture of alum, aluminum chloride or other aluminum salts.

In my co-pending patent application covering a process for the manufacture of titanium metal, I obtain a by-product of alkali metal aluminate solution by the selective leaching of the aluminum from a titanium-aluminum alloy of specified composition. This by-product alkali metal aluminate solution may be mixed with the alkali metal aluminate solution obtained as a filtrate in Step A, and the combined solutions carbonated together to recover aluminum hydroxide and alkali metal carbonate solution. Thus, all of the aluminum used in this process is ultimately recoverable as aluminum hydroxide or alpha-alumina. If purer by-product  $CO_2$  gas is not available, filtered flue gas free of  $H_2S$  and  $SO_2$  may be used for the above-described carbonation.

#### STEP C

The calcium fluoride precipitate obtained in Step A above is reacted with sulfuric acid, according to any of the procedures well known to the art, to produce hydrogen fluoride. Thus, for example, a mixture of the

calcium fluoride precipitate and 66° Bé. sulfuric acid are fed into a rotating retort in the proportions of 1 mole of  $CaF_2$  per 1.3-1.5 moles of  $H_2SO_4$ . The rotating retort is fired by gas or oil, and at the feed end, hydrogen fluoride gas is withdrawn at a temperature of 120° C.—180° C. The gases pass through a dust collector (to remove fine particles of  $CaF_2$  carried over) and thence are drawn into a series of absorption towers where the HF is dissolved in an aqueous medium to obtain aqueous hydrofluoric acid solutions of 5% to 52% HF concentration, although more concentrated solutions may be obtained by recirculation. For the process of this invention, solutions containing 5% to 50% of HF, made from  $CaF_2$  and  $H_2SO_4$  by any of the processes of the art, are suitable. The calcium sulfate residue of these processes, usually containing less than 1% of unreacted  $CaF_2$ , is discharged and discarded.

It is also advisable to add small amounts of acid-grade fluorspar from time to time to the calcium fluoride precipitate from Step A used in this step, to make up for mechanical and other losses in the recycling of reagents through this process. Such losses can be kept below 5% (of the total charge of  $CaF_2$  used) per cycle.

#### STEP D

The aqueous hydrofluoric acid solution (containing 5% to 50% HF) obtained in Step C is now reacted with a member of the group consisting of titanium dioxide, hydrated titanium dioxide and titanic acid, in stoichiometric proportions as is required for the formation of fluotitanic acid.



The titanium compound used may be any suitably pure compound of tetravalent titanium and oxygen. Metallurgical titanium dioxide or rutile may be used. An ideal source of titanium is the hydrated  $TiO_2$  (or titanic acid) obtained by the hydrolysis of the titanic sulfate in the widely practiced Washburn process (U. S. Patent 1,889,027 (1933); British Patent 288,569 (1927)). The titanium compound dissolves readily in the hydrofluoric acid solution, especially on heating for a short period. The hydrated titania dissolves more readily than does the anhydrous or crystalline titani.

The resultant solution of fluotitanic acid is now reacted with a member of the group consisting of the hydroxides, carbonates or bicarbonates of the alkali metals, according to the equation:



The alkali metal carbonate solutions obtained as the filtrate in Step B are ideally suited for this neutralization. When these are so used, the carbon dioxide evolved during the neutralization may be used to effect the carbonation in Step B. However, this process is not limited to the use of the filtrate of Step B in such a manner. A fresh solution of alkali may be employed.

There is thus obtained an aqueous solution containing alkali metal fluotitanate, from which the salt crystallizes on cooling. The most satisfactory recovery is obtained with potassium fluotitanate which is soluble in water to the extent of 1.28% at 20° C. and 0.75% at 5° C. On cooling, almost all of the  $K_2TiF_6$  crystallizes out as the monohydrate. Lithium fluotitanate



and sodium fluotitanate ( $Na_2TiF_6$ ) are considerably more soluble, and may precipitate only incompletely on cooling. It may be necessary to concentrate solutions of these salts to obtain adequate recovery.

After filtering off the alkali metal fluotitanate, the aqueous filtrate may then be divided into two portions. The first portion is returned to the process for use in

Step A as the aqueous medium for the preparation of the milk of lime slurry. The other portion is returned to the process for use in Step C as the aqueous medium for the absorption of the HF gas in the preparation of the hydrofluoric acid solution. In this manner, all of the alkali metal fluotitanate not recovered by cooling, precipitation and filtration in Step D, is recycled to the process and ultimately recovered. Thus, in a preferred embodiment of the process of this invention, the reaction of Step A and the absorption of HF in Step C is effected in an aqueous medium consisting at least in part of the filtrate from Step D, which is a solution of alkali metal fluotitanate saturated at the temperature of the filtration.

The following example is given to define and to illustrate this invention but in no way to limit it to reagents, proportions and conditions described therein. Obvious modifications will occur to any person skilled in the art. All proportions given are parts by weight.

*Example*

A magnesia-lined crucible is charged with 68 parts of molten aluminum metal and 240 parts of anhydrous potassium fluotitanate is added. The mixture is placed in an induction furnace and slowly heated, with agitation, until the reaction is complete and the reaction mixture has obtained a temperature of about 1500° C. The molten reaction mixture is maintained near this temperature for about 15 minutes, and the molten slag (comprising an equimolecular mixture of  $K_3AlF_6$  and  $AlF_3$ ) is then carefully decanted from the regulus of molten titanium-aluminum alloy. The molten alloy is cooled slowly to room temperature. There is thus obtained about 78.0-79.0 parts of an alloy containing about 60% titanium and 40% aluminum.

The molten slag salt mixture, containing 172.2 parts of  $K_3AlF_6$  (0.67 mole) and 56.0 parts of  $AlF_3$  (0.67 mole) is cooled rapidly and solidified. The solid is comminuted and added to a slurry of 171 parts of lime ( $CaO$ ) (3 moles) in 2000 parts of water. (Instead of water in succeeding runs, the filtrate from the final precipitate of  $K_2TiF_6$  may be used here.) The reaction mixture is heated at 95°-100° C. with good agitation for an hour, or until precipitation of  $CaF_2$  is complete. The precipitated calcium fluoride is then filtered off, washed on the filterpress with a small amount of hot water, and the combined filtrate and washings are combined. The filtercake is pressed as free of water as possible.

The combined filtrate and washings from the preceding step are now carbonated at atmospheric temperature, while still hot (i. e. at 50°-90° C.) until a total of 44 parts of carbon dioxide has been absorbed. The precipitated aluminum hydroxide is filtered off, washed on the filterpress with a small amount of hot water, pressed as free of water as possible, and is then calcined at 900°-1100° C. for conversion to alpha-alumina. From 62 to 65 parts of alumina are thus recoverable. The filtrate and washings from the  $Al(OH)_3$  precipitate, comprising a solution of 138 parts of  $K_2CO_3$  in about 2100 parts of water, are retained for subsequent use.

The calcium fluoride filtercake obtained above (containing about 234 parts of  $CaF_2$  (3 moles)) is mixed with 425 parts of 66° Bé. sulfuric acid (4 moles) and heated in a rotary kiln, or by any of the methods well known in the art, to generate hydrogen fluoride gas. The HF gas evolved (120 parts) is absorbed in 1080 parts of water to yield 1200 parts of a 10% w./w. hydrofluoric acid solution. (After the first run, the filtrate from the final precipitate of  $K_2TiF_6$  may be used in place of water to make up this hydrofluoric acid solution. It is also advisable to add to each succeeding batch of  $CaF_2$  filtercake, about 12 parts of acid-grade fluorspar to compensate for mechanical and other losses.)

To the 1200 parts of 10% HF solution (6 moles), add now 80.0 parts of titanium dioxide (1 mole) and heat, with agitation, until the  $TiO_2$  has dissolved. Add

now the solution of 138 parts of  $K_2CO_3$  (1 mole) in 2100 parts of water reserved from the preceding step. Carbon dioxide (44 parts) will be evolved, and may be piped off and used to carbonate a succeeding batch of potassium aluminates solution. On cooling to 5°-10° C., a copious precipitate of  $K_2TiF_6 \cdot H_2O$  settles out. This is filtered off, and dehydrated by drying at a temperature of 150°-200° C. There is thus obtained 210-215 parts of  $K_2TiF_6$  which are returned, with "make-up" to the first step of the process. The filtrate from the  $K_2TiF_6 \cdot H_2O$  precipitate (about 3200 parts of solution containing about 25 parts of  $K_2TiF_6$ ) is divided. Part is used to make up the lime slurry for reaction with the  $K_3AlF_6 \cdot AlF_3$  salt mixture (q. v. supra) and the remainder is used to absorb the HF gas (q. v. supra). By this recycling of the filtrate, the yield of  $K_2TiF_6$  (anhydrous basis) in succeeding batches may be brought to 240 parts per cycle.

A raw materials balance for this process follows:

|                                 |                                 |
|---------------------------------|---------------------------------|
| 68 parts aluminum               | 68 parts aluminum               |
| 171 parts lime                  | 171 parts lime                  |
| 425 parts 66° Bé. sulfuric acid | 425 parts 66° Bé. sulfuric acid |
| 80 parts titanium dioxide       | 80 parts titanium dioxide       |
| 12 parts acid-grade fluorspar   | 12 parts acid-grade fluorspar   |

yield { 78.0-79.0 parts of 60%  
Ti/40% Al alloy  
62-65 parts of alumina

Having described my invention, what I claim and desire to protect by Letters Patent is:

1. A cyclic process for the manufacture of titanium-aluminum alloys and the regeneration of the intermediates of said process which comprises the steps of: (a) reacting an alkali metal fluotitanate with metallic aluminum in stoichiometric excess at advanced temperatures to obtain the said titanium-aluminum alloy and a by-product mixture of alkali metal fluoaluminate and aluminum fluoride, and thereafter separating said alloy from said salt mixture; (b) reacting the mixture of alkali metal fluoaluminate and aluminum fluoride, in an aqueous medium, with lime in quantity sufficient to form a precipitate of calcium fluoride and a solution of alkali metal aluminates, and separating said precipitate from said solution; (c) carbonating the alkali metal aluminates solution with a carbon dioxide-containing gas to form a precipitate of aluminum hydroxide and a solution of alkali metal carbonates, and separating said precipitate from said solution; (d) reacting the calcium fluoride obtained in step (b) with sulfuric acid at advanced temperatures to form hydrogen fluoride gas, absorbing said gas in an aqueous medium and reacting the resultant solution of hydrofluoric acid with a member of the group consisting of titanium dioxide, hydrated titanium dioxide and titanic acid, whereby an aqueous solution of fluotitanic acid ( $H_2TiF_6$ ) is obtained; and (e) neutralizing the fluotitanic acid with a member of the group consisting of the hydroxides, carbonates and the bicarbonates of the alkali metals, recovering the resultant alkali metal fluotitanate and returning the same to the first step of the process.

2. The process of claim 1 for the manufacture of titanium-aluminum alloys containing from 0.1% to 95% of titanium.

3. The process of claim 1 where from 38.5 grams to 47.9 kilograms of metallic aluminum is reacted with each gram-mole of alkali metal fluotitanate.

4. The process of claim 1 where the filtrate from the precipitate of alkali metal fluotitanate is used at least in part as the aqueous medium for the reaction of the alkali metal fluoaluminate-aluminum fluoride with the lime in step (b).

5. The process of claim 1 where the filtrate from the precipitate of alkali metal fluotitanate is used at least in part as the aqueous medium for the absorption of the hydrogen fluoride gas in step (d).

6. The process of claim 1 where the filtrate from step (c) containing alkali metal carbonates is employed to neutralize the fluotitanic acid in step (e).

7. The process of claim 1 where the carbon dioxide evolved during the reaction of fluotitanic acid with an

alkali metal carbonate in step (e) is employed to carbonate the alkali metal aluminates solution in step (c).

8. The process of claim 1 where the alkali metal fluotitanate is potassium fluotitanate.

9. The process of claim 1 where the alkali metal fluotitanate is sodium fluotitanate.

10. The process of claim 1 where the alkali metal fluotitanate is lithium fluotitanate.

11. The process of claim 1 where the reaction of the alkali metal fluotitanate and metallic aluminum is effected within a temperature range of 660° C. to 1800° C.

12. The process of claim 1 where the reaction mixture of the alkali metal fluotitanate and metallic aluminum is brought to a terminal temperature within the range of 1100° C. to 1750° C.

13. The process of claim 1 where the reaction mixture

5

10

15

of the alkali metal fluotitanate and metallic aluminum is brought to within a terminal temperature range at which both the end-product regulus of titanium-aluminum alloy and by-product slag are in the molten state.

References Cited in the file of this patent

UNITED STATES PATENTS

1,648,954 Marden ----- Nov. 15, 1927

OTHER REFERENCES

Comprehensive Treatise on Inorganic and Theoretical Chemistry, vol. 5, pages 289 and 306; vol. 2, page 127; vol. 7, page 69. Edited by Mellor. Pub. in 1927 by Longmans, Green and Co., New York.

Journal of Metals, June 1952, page 612. Pub. by the A. I. M. E., New York.